

# UNITED STATES PATENT OFFICE.

ROYALE HILLMAN STEVENS, OF RISDON, HOBART, TASMANIA, AUSTRALIA, ASSIGNOR  
TO ELECTROLYTIC ZINC COMPANY OF AUSTRALASIA, PROPRIETARY LIMITED, OF  
MELBOURNE, VICTORIA, AUSTRALIA.

## RECOVERY OF ZINC BY ELECTROLYSIS.

1,322,071.

Specification of Letters Patent. Patented Nov. 18, 1919.

No Drawing.

Application filed May 6, 1919. Serial No. 295,307.

*To all whom it may concern:*

Be it known that I, ROYALE HILLMAN STEVENS, a citizen of the United States of America, residing at Risdon, Hobart, in the State of Tasmania, Commonwealth of Australia, have invented certain new and useful Improvements in the Recovery of Zinc by Electrolysis, of which the following is a specification.

10 This invention relates to certain improvements in the recovery of zinc by electrolysis and refers more especially to the electro-deposition of zinc from zinc sulfate solutions obtained by leaching ores, concentrates or other zinc bearing material with sulfuric acid (or spent electrolyte).

20 In the recovery of zinc by electrolysis the presence of certain impurities interferes with and detrimentally affects the deposition of zinc and for effective working it is very desirable that such impurities should be removed especially in view of the fact that the said impurities accumulate with the continuous circulation of the solutions. 25 Some of the substances which thus adversely affect the electro-deposition of the zinc are present in very small quantities (e. g. cobalt) and the usual methods of purification (with limestone and zinc dust) have not been found effective for their elimination.

30 I have discovered that if during the electrolysis of the zinc sulfate solutions there is present a certain small proportion of glue the deleterious effect of such impurities upon the electro-deposition of the zinc is materially minimized and operations can be continued with effective results in the presence of glue under conditions which would otherwise not be possible.

40 I am aware that glue has been used in the electro-deposition of lead for the purpose of obtaining a smooth coherent deposit but it is generally recognized in the electro-deposition of zinc that glue does not have this effect and is therefore not required. So

far as I am aware it has not been the practice to employ glue in the electro-deposition of zinc nor has it been known that the presence of glue would have any action in retarding or checking the deleterious effect of 50 certain impurities (such as cobalt) not otherwise easily removable upon the deposition of the zinc.

55 In adapting this invention to the current practice in the electro-deposition of zinc I add a certain small proportion of glue in solution either to the electrolyte before passing into the cells or to the electrolyte in the cells. The amount of glue added is determined by the amount of impurities present in the solution, and such amount increases as the impurities increase within limits owing to the continuous circulation of the solutions. Moreover when manganese is present in the electrolyte in the form of 65 manganese sulfate a scale of manganese dioxid is formed on the anodes which in the presence of glue is deposited in more coherent form which inhibits corrosion of the anodes. 70

I claim—

1. In the recovery of zinc by electrolysis, the step of reducing the prejudicial effect upon the electro-deposition of the zinc of the presence of cobalt and/or nickel by the addition of glue to the electrolyte prior to electrolysis; substantially as described. 75

2. In the recovery of zinc by electrolysis, the step of reducing the prejudicial effect upon the electro-deposition of the zinc of the presence of cobalt and/or nickel by the addition of an animal colloid to the electrolyte prior to electrolysis; substantially as described. 80

85 In witness whereof I have affixed my signature in presence of two witnesses.

ROYALE HILLMAN STEVENS.

Witnesses:

EDWARD H. BUTLER,  
ALLAN MCINTYRE.